

## UNITED STATES PATENT OFFICE.

ALVAH W. CLEMENT, OF CLEVELAND, OHIO, ASSIGNOR, BY MESNE ASSIGNMENTS, TO LUDLUM STEEL CO., OF WATERVLIET, NEW YORK, A CORPORATION OF NEW JERSEY.

## METALLIC ALLOY.

No Drawing.

Application filed August 15, 1917. Serial No. 186,267.

*To all whom it may concern:*

Be it known that I, ALVAH W. CLEMENT, a citizen of the United States, residing at Cleveland, in the county of Cuyahoga and 5 State of Ohio, have invented a certain new and useful Improvement in Metallic Alloys, of which the following is a full, clear, and exact description.

This invention relates to an alloy which 10 may be used for the fabrication of articles and devices which in their use are subjected to the action of hot corroding gases, and high temperatures, as, for example, annealing and carburizing boxes, saggars, which 15 are used under conditions involving high temperatures, crucibles for melting brass, bronzes, etc., parts of furnaces, or in fact in any situation where it is desired to produce an article which is resistant to heat and 20 to corrosion and, in modified form, may be used for the making of non-corrosive forged articles, such as dies for die castings, ball races and balls for ball bearings, and other articles.

25 The alloy comprises a combination of iron, chromium and titanium, which combination when alloyed has a high melting point, is tough, and not brittle.

To the alloy of the elements mentioned, 30 small proportions of silicon, or of silicon with aluminum may be added, which prevent material oxidization of the surfaces of an article fabricated of the alloy, by providing a film or surface of oxide which serves 35 as a protecting covering.

In making the alloy, the carbon content should be kept as low as possible, as by the use of oxidizing slags, for carbon in appreciable amounts renders the alloy hard and 40 very difficult to work.

A very effective alloy for the purposes I have found to consist of the following; titanium 6 per cent, chromium 10 per cent, aluminum 10 per cent, the balance of iron 45 and silicon, the silicon present being less than 1 per cent. The percentage of aluminum and titanium may be varied, but should not be less than 5 per cent of each of the elements mentioned. The chromium may 50 vary from 10 per cent to 30 per cent, the iron and silicon always making up the balance of the alloy.

If desired, molybdenum may be added where the percentage of titanium present is

above 5 per cent, but is undesirable with 55 lower percentages of titanium. Where molybdenum is so added, the percentage of titanium must be maintained sufficiently high so that the addition of molybdenum will not make an inherently soft alloy. The 60 molybdenum imparts to the alloy the property of easy machinability.

Where the alloy is intended to be used under conditions involving very high temperatures, the percentage of titanium can be 65 carried close to 20 or 25 per cent, the chromium being maintained at approximately 15 per cent.

Inasmuch as the alloy is non-warping, even at high temperatures, it is possible to 70 construct articles of this alloy to have thin walls, and generally the quantity of metal required in forming the articles is much less than with many other metals because of this non-warping property, which enables the use 75 of light weight structures.

The alloy may be prepared by directly melting the elements forming the alloy. It is preferable to form the alloy using as the sources of the elements ferro-titanium and 80 ferro-chromium. When utilizing these sources of ingredients the same are preferably melted in the electric furnace together with suitable fluxes, which fluxes are those well known in the art.

The alloy may be very advantageously used for the making of dies for die castings, or for dies and plungers in the handling of hot glass, or for molds in the handling of hot glass, as well as for forming ball bearings, by fabricating the articles thus to be used of the alloy described, and subsequently heat treating the surfaces which are to be exposed to the wear and abrasion, as by carburizing so as to form at these surfaces a high 95 proportion of carbides which will comprise carbides of titanium and chromium. The carbides mentioned are exceedingly hard and resistant to wear and abrasion.

Having described my invention, what I 100 claim is:

1. A substantially nickel free alloy resistant to corrosion and to oxidation at high temperatures, containing on analysis approximately 5% to 25% of titanium, and the 105 balance principally iron and chromium.

2. A substantially nickel free alloy, resistant to corrosion and to oxidation at high

temperatures, containing on analysis chromium not to exceed 30%, titanium not to exceed 25%, and the balance principally iron.

3. A substantially nickel free alloy resistant to corrosion and to oxidation at high temperatures, and containing on analysis chromium not below 10% and not to exceed 30%, titanium not to exceed 25%, and the 10 balance principally iron.

4. A substantially nickel free alloy resistant to corrosion and to oxidation at high temperatures containing on analysis 5% to 25% of titanium, substantially 10% to 30% 15 of chromium, the balance consisting principally of iron.

5. An article resistant to corrosion and to oxidation at high temperatures made of a substantially nickel free alloy containing on 20 analysis titanium from 5% to 25%, the balance being principally chromium and iron, the exposed surface of the article containing carbides of the principal ingredients of the alloy.

25 6. An article resistant to corrosion and to oxidation at high temperatures made of a substantially nickel free alloy containing on analysis 10% to 30% of chromium, titanium not to exceed 25%, the balance being principally iron, the exposed surface of the article containing carbides of aforesaid ingredients.

30 7. A substantially nickel free alloyed soft steel resistant to corrosion and to oxidation 35 at high temperatures containing on analysis

approximately 5% to 20% of titanium, and the balance principally iron and chromium.

8. A substantially nickel free alloyed soft steel resistant to corrosion and to oxidation at high temperatures containing on analysis 40 chromium not to exceed 30%, and titanium not to exceed 20%.

9. A substantially nickel free alloyed soft steel resistant to corrosion and to oxidation at high temperatures containing on analysis 45 chromium not below 10% and not to exceed 30%, and titanium not to exceed 20%.

10. A substantially nickel free alloyed soft steel resistant to corrosion and to oxidation at high temperatures containing on 50 analysis 5% to 20% of titanium, and substantially 10% to 30% of chromium.

11. An article resistant to corrosion and to oxidation at high temperatures made of substantially nickel free alloyed soft steel 55 containing on analysis titanium about 5% to 25%, the balance being principally chromium and iron, the exposed surface of the article containing carbides of the principal ingredients of the alloy.

12. An article resistant to corrosion and to oxidation at high temperatures made of substantially nickel free alloyed soft steel containing on analysis chromium about 10% to 30%, and titanium not to exceed 20%, the 60 exposed surface of the article containing carbides of aforesaid ingredients.

In testimony whereof, I hereunto affix my signature.

ALVAH W. CLEMENT.